

March 19, 1935.

A. PATERSON

1,994,662

METHOD OF ROLLING SHEET METAL PACKS

Filed June 1, 1934

Fig. 1.



Fig. 2.



Fig. 3.



Fig. 4.

Fig. 5.



INVENTOR  
Alexander Paterson  
BY  
John S. Powers  
ATTORNEY

## UNITED STATES PATENT OFFICE

1,994,662

## METHOD OF ROLLING SHEET METAL PACKS

Alexander Paterson, Buffalo, N. Y.

Application June 1, 1934, Serial No. 728,545

4 Claims. (Cl. 29—19)

This invention relates to the reduction of sheet metal and more particularly involves a novel process of pack rolling.

In the reduction of sheet metal by pack rolling various factors, which determine the shape of the pack and the individual sheets thereof, are involved. These factors include the initial shape and temperature of the pack, the permissible distortion or change in the cross-section or shape 10 of the individual sheets in the pack during the rolling operations, the contour of the rolls and of the working pass provided thereby and the resiliency of the rolls or their resistance to deflection. In order to counteract roll deflection, 15 which is caused by the bending stresses set up during the rolling operations and which is greatest at the central zones of the working rolls, it is the practice to increase the diameter of the rolls at their central zones. Preferably the increase 20 in the diameter of the central zones of the rolls is limited so that during the initial heavy reductions the rolls provide a working pass of convex cross-section while during the succeeding lighter reductions the working pass approaches 25 a cross-section which is substantially flat or rectangular. In other words, the cross-section of the working pass is dependent upon the magnitude of the reduction. Heretofore, owing to the difficulty encountered in fitting a pack to 30 the various sets of the rolls of a tandem or continuous mill with such accuracy as to insure maintenance of the distortion of the individual sheets within the permissible zone of tolerance, it has been the practice to effect the successive 35 reductions by passing and repassing the pack through the rolls of a single stand mill. This mode of procedure is preferable in the case of pack rolling as it eliminates the difficulties attendant upon the accurate fitting of the pack to 40 various sets of working rolls, it being understood in this connection that unless the pack fits the pass provided by the working rolls within a narrow range of tolerance the various sheets of the pack will be distorted and cannot be separated 45 without injury. In the ordinary mill the pack, after being heated, is given four or five passes between the rolls of the stand, the screws being set between passes to regulate or control the magnitude of the reductions. The greatest reduction is obtained in the first pass, the screws being adjusted for this pass so that the reduction obtained corresponds to the maximum permissible deflection of the rolls. In the succeeding passes the screws of the stand are adjusted so 50 that the magnitude of the deflection of the rolls is progressively decreased to decrease the convexity of the pack correspondingly and cause it to approach a flat or rectangular cross-section. It will be apparent, therefore, that after the first 55 pass the magnitude of the screw adjustment is

determined to a large degree by the resiliency of the rolls. Thus substantially the entire capacity of the stand for each series of reductions is utilized in the first pass whereas in the succeeding passes only a fraction of the capacity of the stand is availed of owing to the fact that the roll factors, which are predetermined to effect the greatest reduction in the first pass, remain substantially constant. The magnitude of the reductions, therefore, progressively decreases. Any 10 attempt to effect reductions in the succeeding passes equal in magnitude to those in the first pass would, therefore, result in distortion of the individual sheets beyond the permissible zone of tolerance. Owing to the rapidity at which the 15 pack cools the decrease in the magnitude of the reductions cannot be compensated by increasing the number of passes as after four or five passes the amount of reduction obtained in a single stand of rolls without reheating is practically 20 negligible.

The principal object of the present invention is to overcome the above objections, this object 25 contemplating a novel method of rolling whereby, with respect to a single heating, a maximum reduction of the pack is obtained without injury to the individual sheets thereof.

A further object is a process which can be carried out by existing equipment.

The invention is illustrated in the accompanying drawing in which:

Figure 1 is a view partially in elevation and partially in section of a mill for carrying out my process.

Figure 2 is an exaggerated diagrammatic view 35 illustrating the shape of the pack and the working rolls during the first pass.

Figure 3 is a similar view illustrating the shape of the pack and the working rolls during the third pass.

Figure 4 is a graphic illustration of the magnitude of the reductions obtained in the stands of the mill shown in Fig. 1.

Figure 5 is a view in elevation of a three-stand mill for carrying out my process.

One form of mill for carrying out my process is illustrated in Figure 1. The mill, as illustrated, comprises primary and secondary stands 5 and 6, respectively. Each stand includes upper and lower working rolls 7 and 8, respectively, and a backing roll 9 which co-operates with the lower working roll. The various rolls are mounted in suitable housings 10, each of which is provided with conventional adjusting screws 11 by means of which the magnitude of the reductions is regulated or controlled. The backing rolls 9 are of the kind covered by my Patent No. 1,953,190 issued April 3, 1934, and as illustrated, are formed or provided with end collars 12 and intermediate collars 13, the latter preferably being of a suit- 55

ably smaller diameter than the former. The collars are adapted to co-operate with the associated working roll to limit the deflection of the latter so that during passage of a pack between the 5 working rolls it will be formed with a predetermined cross-sectional convexity. The pressure exercised by the backing rolls upon the associated working rolls, and hence the degree of deflection of the latter, depends among other factors upon 10 the relative diameters of the end and intermediate collars 12 and 13, respectively. It will be apparent, therefore, that the deflection of the working rolls may be regulated to form a pack with a predetermined cross-sectional convexity by 15 varying the relative diameters of the said collars. For example, by increasing the diameter of an intermediate collar 13 of a backing roll or by decreasing the diameters of the end collars 12 or by effecting both of these variations simultaneously, the degree of deflection of the central zone of the associated working roll will be reduced with a corresponding reduction in the cross-sectional convexity of the pack. As noted in my 20 said Patent No. 1,953,190 the variations necessary in the diameters of the collars to obtain the necessary amount of control will for most purposes be of the order of a few thousandths of an inch and such variations can, therefore, be readily obtained by the use of suitable heating and cooling 25 devices.

The primary stand of rolls 5 is preferably a hot mill and is designed with reference to the initial shape of the pack which is to be reduced, that is to say the factors which determine the magnitude 30 of the reductions and the cross-sectional contour of the pack are predetermined to effect, in the first pass, the maximum permissible deflection of the working rolls (see Figure 2), and hence the maximum permissible reduction of the pack. Assuming, for example, that the factors involved 35 are predetermined with respect to a four-sheet pack having an initial thickness of .250" and that the said pack is to be reduced to a thickness of .084", then in the first pass between the working rolls of the stand 5, approximately 42% of the total amount of reduction will be effected (see curve 14 of Figure 4). Approximately 21% of the total reduction will be effected in the second pass while approximately 10.8% and 5.4% 40 would be effected in the third and fourth passes, respectively, in the said stand. It will be apparent that while in the first pass the maximum capacity of the stand is utilized, this cannot be done in the succeeding passes as the deflection of 45 the working rolls must be progressively decreased in order to prevent distortion of the individual sheets of the pack. In the fourth pass the thickness of the pack would be reduced to approximately .117" and the pack would be formed with a cross-section which is substantially 50 flat or rectangular. Hence regardless of the number of additional passes further reductions could not be obtained without reheating and re-rolling the pack. In progressively decreasing the 55 degree of deflection of the working rolls as described, the magnitude of the reductions are correspondingly reduced. Thus, whereas in the first two passes 70% of the total required reduction is obtained only 16.2% of the total reduction could be obtained in the final two passes in the same stand. In order, therefore, to reduce the pack to the desired thickness, i. e., .084", it would be necessary to first reheat it and then further roll it.

In carrying out my process a pack 15 of the 70 dimensions above noted after being heated in

any suitable manner is passed twice between the working rolls of the stand 5, thereby effecting two major reductions or approximately 70% of the required reduction, the diameters of the collars 12 and 13 of the backing roll 9 being regulated or controlled so that the said pack is formed with a predetermined cross-sectional convexity in its second pass between the working rolls. Immediately thereafter, and without reheating, the pack is passed and repassed between the working 10 rolls of the adjacent secondary stand 6, the number of such passes being determined by the amount of reduction to be effected in this stand and in the example given being four. The secondary stand may be either a hot mill or cold 15 mill such as, for example, a watermill, and the rolls thereof are adapted to provide a series of reducing passes which are flatter, that is to say less convex, than the corresponding passes of the series provided by the working rolls of the stand 20 5. The secondary stand of rolls 6 is designed with reference to the shape of the pack 15 as modified by the rolls of the stand 5 in order that two major reductions will be obtained in the first two passes, the collars 12 and 13 of the backing 25 roll 9 providing means for regulating or controlling the cross-sectional contour of the working pass so that it may be made to conform to the changed shape of the pack. In this connection it is understood, of course, that the degree of 30 deflection of the working rolls is small and that the deflection shown in Figures 2 and 3 is greatly exaggerated in order to render the illustrations more clear. The roll factors of the secondary stand being predetermined with respect to the 35 shape or cross-section of the pack as modified by the rolls of the first stand, the maximum permissible deflection of the working rolls is obtained, and hence the maximum permissible reduction of the pack is effected in the first pass. In this 40 pass approximately 20% of the total reduction is effected (see curve 16 of Figure 4). In the second pass approximately 14% of the total reduction is effected while in the third and fourth passes the pack is reduced approximately 10% and 5%, 45 respectively, of the total amount required. In the final pass the pack is reduced to the required thickness, i. e., .084", the total reduction being effected, therefore, in six passes and requiring only one heating of the pack.

It will be apparent upon comparing curves 14 and 16 that whereas approximately 17.3% of the total amount of reduction of the pack is obtained in the first pass in the secondary stand 6 only approximately 10.8% could have been obtained 50 as a third pass in the primary stand 5; that whereas approximately 10% of the total reduction is obtained in the second pass in the secondary stand only approximately 5.4% could have been obtained as a fourth pass in the primary stand; and that whereas approximately 9% of the total reduction is obtained in the final two passes in the secondary stand no equivalent reduction could be obtained in the primary stand without reheating the pack owing to the exhaustion of the resiliency of the working rolls. In other words, by following the procedure described approximately 28.2% greater reduction is obtained, in the example given, than would be obtained upon a single stand mill with a single 55 heating of the pack.

In order to decrease the time between passes and thereby reduce heat losses by radiation the leading end of the pack may, as it emerges from between the working rolls of a stand, be guided 60

back over the top roll thereof so that in the succeeding pass in the stand it becomes the trailing end of the pack. Any suitable apparatus may be employed for this purpose. For example, 5 as the pack emerges from the rolls it may be directed by a guide over the top of the upper working roll, the leading end being engaged by a magnetic roller which returns the pack to a point from which it may be reintroduced between the 10 rolls as described.

A modified form of mill for carrying out the process is shown in Figure 5. The mill, as illustrated in this embodiment, includes a primary stand 17 and secondary stands 18 and 19. Each 15 of the said stands includes upper and lower working rolls 20 and 21, respectively, and backing rolls 22 which are associated with the lower working rolls. The backing rolls 22 are formed or provided with end collars 23 and intermediate collars 24, the said collars co-operating with the associated working rolls to regulate or control the degree of deflection of the latter as described in connection with the mill shown in Figure 1. The stand 17 is similar to the stand 5 of the mill 20 shown in Figure 1 while the stands 18 and 19 are both similar to the stand 6 of the said mill.

In carrying out the process the first pack to be reduced is passed between the working rolls of the primary stand 17 to effect two major reductions. Thereafter the said pack is immediately 30 introduced between the working rolls of either of the adjacent secondary stands 18 and 19 while a second pack is introduced between the working rolls of the primary stand 17. Upon completion 35 of the two major reductions of the second pack in the primary stand 17 and while the first pack is receiving its third pass, or minor reduction, the said second pack is introduced immediately between the working rolls of the other of the 40 secondary stands. The use of three stands in the manner described, therefore, has the advantage that the primary stand 17 may be worked continuously, which, of course, cannot be done where only two stands are employed as only two passes 45 are made in the primary stand while in many cases four passes will be made in the secondary stand. When the packs are formed of two or three sheets, the individual sheets may, if desired, be first given a single pass through the 50 rolls of the primary stand 5 and then piled and given one or two passes through the rolls of the said stand prior to the rolling of the packs in the secondary stand 6.

From the foregoing it will be apparent that the 55 practice of the process enables a substantially greater reduction of a pack, with respect to a single heating, than can be obtained by conventional rolling methods. Moreover, distortion or injury to the individual sheets of the pack is 60 avoided owing to the predetermination of the roll factors and the accurate control of roll deflection by the collars of the backing rolls. The backing rolls of the mills shown in the two embodiments described may be substituted for the conventional 65 backing rolls of standard mills. The process, therefore, has the further advantage that its practice may be carried out with existing mills, the latter being readily adaptable to the present method.

70 Having fully described my invention, I claim:  
 1. The method of rolling a sheet metal pack to 75 reduce it to a predetermined thickness and cross-sectional contour, which method consists in passing the pack at least twice through a stand of rolls having roll factors predetermined with re-

spect to the initial shape or cross-section of the pack, whereby to effect two major reductions while forming the pack with a predetermined cross-sectional convexity and passing and re-passing the pack through a second stand of rolls having roll factors predetermined with respect to the shape or cross-section of the pack as modified in the last pass through the rolls of the first stand, whereby to effect in the second stand two major reductions in the first two passes and such 10 minor reductions in the succeeding passes as may be required to reduce the pack to the thickness and cross-sectional contour which has been predetermined.

2. The method of rolling a sheet metal pack to 15 reduce it to a predetermined thickness and cross-sectional contour, which method consists in heating the pack, passing it twice through a stand of rolls having roll factors predetermined with respect to the initial shape or cross-section of the 20 pack, whereby to effect two major reductions while forming the pack with a predetermined cross-sectional convexity and passing and re-passing the pack without reheating through a second stand of rolls having roll factors predetermined with respect to the shape or cross- 25 section of the pack as modified in the second pass through the rolls of the first stand, whereby to effect in the second stand two major reductions in the first two passes and such minor 30 reductions in the succeeding passes as may be required to reduce the pack to the thickness and cross-sectional contour which has been predetermined.

3. The method of rolling a sheet metal pack 35 to reduce it to a predetermined thickness and cross-sectional contour, which method consists in heating the pack, passing it twice through a stand of rolls having roll factors predetermined with respect to the initial shape or cross-section 40 of the pack, whereby to effect two major reductions while forming the pack with a predetermined cross-sectional convexity and passing and re-passing the pack, without reheating, at least 45 three times through a second stand of rolls having roll factors predetermined with respect to the shape or cross-section of the pack as modified in the second pass through the rolls of the first stand, whereby to effect in the second stand two major reductions in the first two passes and one 50 minor reduction in the succeeding pass and thereby reduce the pack to the thickness and cross-sectional contour which has been predetermined.

4. The method of rolling a sheet metal pack to 55 reduce it to a predetermined thickness and cross-sectional contour, which method consists in heating the pack, passing it twice through a stand of rolls having roll factors predetermined with respect to the initial shape or cross-section of the 60 pack, whereby to effect at least 40% of the total amount of reduction required and at the same time forming the pack with a predetermined cross-sectional convexity and passing and re-passing the pack, without reheating, through a second 65 stand of rolls having roll factors predetermined with respect to the shape or cross-section of the pack as modified in the second pass through the rolls of the first stand, whereby to effect in the second stand two major reductions in the first 70 two passes and such minor reductions in the succeeding passes as may be necessary to reduce the pack to the thickness and cross-sectional contour which has been predetermined.